

R. GAHL.  
FLOTATION APPARATUS.  
APPLICATION FILED JAN. 29, 1918.

1,401,598.

Patented Dec. 27, 1921.



Inventor  
Rudolf Gahl  
By Raynes Townsend & Brickner  
Attorneys

# UNITED STATES PATENT OFFICE.

RUDOLF GAHL, OF MIAMI, ARIZONA, ASSIGNOR, BY MESNE ASSIGNMENTS, TO PNEUMATIC PROCESS FLOTATION COMPANY, OF NEW YORK, N. Y., A CORPORATION OF DELAWARE.

## FLOTATION APPARATUS.

1,401,598.

Specification of Letters Patent. Patented Dec. 27, 1921.

Application filed January 29, 1918. Serial No. 214,318.

To all whom it may concern:

Be it known that I, RUDOLF GAHL, a citizen of the United States, residing at Miami, in the county of Gila and State of Arizona, have invented certain new and useful Improvements in Flotation Apparatus, of which the following is a specification.

My invention relates to an improved apparatus for use in the concentration of ores by what is now known in the art as "flotation" or the process by which the valuable minerals in a mass of finely ground ore are caused to float on a liquid with which the finely ground ore is associated; and particularly relates to an apparatus for use in froth flotation in which the minerals floated gather in and on the surfaces of bubbles of air or gas forced through the pulp or ore-carrying liquid.

In carrying out this air-flotation process, where the main bulk of the ore is composed of very finely ground particles, *i. e.* "slimes," I have found that it is important to maintain a certain percentage of granular material, *i. e.* "sands," in the pulp; and the present application relates to means for so conducting the process as to best make use of this percentage of coarse material by modifying the consistency of a pulp-body of the kind above referred to in the course of the operation.

In flotation tanks provided with perforated bottoms through which the mass of pulp flows, the mixing of the coarse and fine pulp particles resulting from the injection of air through the porous bottom is not complete, and there is a certain amount of stratification *i. e.* the lower layers will contain a greater percentage of the larger grains, the ratio of liquid to solid matter being therefore lower and the pulp relatively denser in this layer.

There are now in use pneumatic flotation machines, which utilize baffles having their lower edges spaced from the bottom of the machine. In this manner eddy-currents are formed near the bottom which have the effect of moving the sand particles relatively fast, and are for this reason perhaps responsible for the shortcomings of such machines in that a low recovery of the coarser particles is thus effected. Such eddy-currents were, however, thought to be essential for the smooth operation of such machines

whenever the bottom was horizontal or had only a gentle slope.

I find now that eddy-currents are not necessary and can be dispensed with by providing baffles which reach clear down to the bottom of the flotation machine, and are provided with openings or perforations in such a manner that an even stream of pulp results.

A further advantage of this mode of operation is that the granular material is subjected to flotation treatment in the form of a thicker pulp, while the slimy material is treated as a more dilute pulp, both forms of the material being therefore subjected to the action of the air bubbles in the manner best adapted for more complete flotation concentration.

The invention will be more clearly understood from the accompanying diagrammatic drawings in which—

Figure 1 is a longitudinal cross-section of a flotation tank, the usual details of construction being omitted;

Fig. 2 is a like cross-section showing several modifications;

Fig. 3 shows a cross-section of a modified form; and

Fig. 4 shows in elevation one of the partitions used in Fig. 3.

Referring to Fig. 1, the porous bottom may be of any of the well-known constructions in which air under pressure is forced through a perforated diaphragm 2, into the mass of ore pulp. I prefer to use the form of bottom described and illustrated on pp. 611 and 612 of vol. 55 of the *Transactions of the American Institute of Mining Engineers* for 1916, which briefly stated comprises removable air-chambers having porous tops 2, air under pressure being introduced into the chambers through pipes 50, Fig. 1. Arranged at suitable intervals, and extending upward from the porous diaphragms are baffles 3, 3, 4 is the front-line over which the froth flows in the well-known manner.

In case it is desired to subdivide the tank into compartments, perforated partitions may be used. Thus at 6, Fig. 2, is shown a partition having a slot 7, extending substantially across the tank, through which the pulp flows from one compartment to the next, the bottom of the slot being a con-

siderable distance, *e. g.* from 12 to 20 inches above the porous diaphragm.

At 8, is shown a partition having several slots containing guiding lips 9. At 10 and 5 11 are shown other forms of lips, all these forms of lips being preferably so shaped as to downwardly direct the flow of pulp from one compartment to the next. In Fig. 10 2, the direction of flow of the ore pulp through the tank is indicated by the arrow 12.

In the form of apparatus shown in Figs. 3 and 4, the partition 30 is shown as provided with a series of perforations 31. In 15 operation, the pulp, prepared for flotation by admixture of a suitable frothing agent, is delivered into the tank at one end through the conduit 15, flows over the porous bottom, and is delivered at the other end preferably over a weir 16, to the delivery conduit 17. An upwardly directed air jet 27 may be used at this point to keep the passage 19 open and to assist the flow of pulp through the tank.

25 As above pointed out, the air-bubbles passing up through the perforated diaphragm 2 do not effect a complete mixing of the coarser and finer particles of the pulp, the coarser particles tending to form an underlying stratum of relatively thicker pulp, which is first subjected to the flotation reaction. The forward movement of this underlying stratum is delayed by the baffles 3, 3, (Fig. 1) or by the perforated partitions, located at suitable distances apart, so that ample time for their effective flotation is given. The thinner or more dilute overlying portion is also subjected to the action of the rising air bubbles and is thus also treated in the best condition, since, as is well-known, slimy pulp is best treated when largely diluted.

45 The bottom of the tank may be horizontal or inclined. Even with a horizontal bottom, there will be no trouble with sand blanketing the porous diaphragm, as long as this diaphragm is kept in good working order.

In the arrangements shown in Figs. 2, 3 50 and 4, the partitions prevent the froth from moving from one compartment to the next, while the openings therethrough provide a free passage of the tailings from each compartment to the next one.

The number and arrangement of the openings 55 is such as to cause the pulp to flow in an even stream. The result of this construction is that in long machines having a more or less inclined bottom, the level of the pulp in each successive compartment 60 will be lower than that above it, so that the depth of pulp in each compartment will be essentially the same throughout the whole length of the machine.

The various forms of guiding lips shown 65 have the common feature that they force the

pulp moving from one compartment to the next to take a somewhat downward course through which it is not likely that mineral particles made buoyant by attached air-bubbles will follow. Such buoyant mineral particles will, on the contrary, be unobstructed in their natural upward course.

As an example of practical operation, I will refer to a test made in a concentrating plant, the flow-sheet of which is briefly as 75 follows:

The ore after having been ground to a suitable fineness by a combination of rock-crushers and ball-mills and having been "oiled" in the ball-mills is passed to flotation machines. The tailings from the flotation machines are separated into a sand and a slime product by a drag classifier, the sand-product going to waste after re-treatment on tables, and the slime products going to 85 waste directly.

The test in question was made with two sections of this plant. The flotation equipment of a section consists of a rougher machine containing in parallel two rows of ten 90 compartments provided with the slotted partitions illustrated at 6 in Fig. 2. The rougher concentrate is re-treated on a cleaner machine consisting of two rows of six compartments each of somewhat smaller dimensions. While the cleaner concentrate represents a finished product, the cleaner tails are returned to the rougher machine.

Several thousand tons of ore were treated in the manner described, and the following 100 figures represent the principal results of a twenty-four hour run:

|                       |                  |                  |
|-----------------------|------------------|------------------|
| Tonnage treated       | 1516.4 tons.     | 1516.4 tons.     |
| Fineness of grinding  | 4.3% on 48 mesh. | 4.3% on 48 mesh. |
| Feed assay            | 1.00             | sulfid copper.   |
| Slime tailing         | .11              | on 48 mesh.      |
| Sand tailing          | .14              | "                |
| Flotation concentrate | 32.30            | "                |
| Table concentrate     | 15.78            | "                |

I claim:

1. An apparatus for ore pulp concentration comprising a tank having a porous bottom impermeable to the downward passage therethrough of ore pulp, means for forcing gas therethrough, partitions subdividing the tank into compartments, said partitions extending to and being imperforate in immediate proximity to the bottom of the tank and provided with openings above said bottom, said openings being in such number and arrangement as to cause the pulp to flow in an even stream. 110

2. An apparatus for ore pulp concentration comprising a tank having a porous bottom impermeable to the downward passage therethrough of ore pulp, means for forcing gas therethrough, and partitions subdividing the tank into compartments, said partitions extending to and being imperforate in immediate proximity to the bottom of the tank and provided with openings above said bottom, said openings having lips 115

arranged to guide the pulp downwardly in its passage through said openings.

3. A long straight-line flotation cell having a porous bottom impermeable to the downward passage therethrough of ore pulp, means for forcing gas through said porous bottom, and partitions subdividing the cell

into compartments, said partitions extending to the bottom of the cell and provided with openings spaced and distributed above said bottom.

In testimony whereof, I affix my signature.

RUDOLF GAHL.